

## UNITED STATES PATENT OFFICE

VIGGO DREWSSEN, OF LARCHMONT, NEW YORK, ASSIGNOR, BY MESNE ASSIGNMENTS, TO BRADLEY-MCKEEFE CORPORATION, OF NEW YORK, N. Y., A CORPORATION OF NEW YORK

## MONOSULPHITE WOOD TREATING PROCESS AND RESULTING FIBER AND PAPER

No Drawing.

Application filed January 29, 1925. Serial No. 5,636.

This invention relates to processes of treating either deciduous or coniferous woods with soluble monosulphite liquor, the monosulphite being used in sufficient quantities to keep the reaction slightly alkaline throughout the digesting operation, and being substantially the only digestive reagent employed. It also comprises the peculiar pulp and paper resulting from such a process. 10 This application is a continuation of my previous applications, Serial No. 474,970, filed June 4, 1921, and Serial No. 623,513, filed March 7th, 1923. This invention has been in commercial use by my authority and under 15 my directions for some time, the present daily output of pulp exceeding forty tons, and preparations being under way to increase the production still further. Monosulphites suitable for the purpose include 20 sodium, potassium and magnesium monosulphites, the first being most conveniently employed. Solutions of all these monosulphites are substantially neutral and are slightly alkaline in their reaction toward 25 litmus. My process is so conducted that the cooking liquor preserves these substantially neutral, slightly alkaline characteristics throughout the digesting operation.

I am aware that various processes involving the use of more or less soluble monosulphite have been frequently mentioned in 30 patents and publications for the treatment of vegetable fibers, ever since the publication of the Cross British Patent No. 4,984 of 35 1880. But so far as I am aware, no commercially valuable process for the treatment of wood by a monosulphite process was ever devised prior to my invention of the process herein described and claimed. I myself succeeded 40 in devising a monosulphite process suitable for the treatment of cornstalks, bagasse and other straws, which is described and claimed in my U. S. Patent No. 1,229,422. But that particular process is not 45 applicable to the treatment of wood without the modifications hereinafter described and claimed. Moreover, the fibers resulting from the treatment of cornstalks, bagasses, etc., as described in my aforesaid patent are of 50 quite different character from those result-

ing from the present process, as hereinafter described and claimed.

My process is based on the discovery that when either coniferous or deciduous woods are digested with soluble monosulphite cooking liquor, the non-cellulosic incrustations of the wood, including lignin, hemicellulose, etc. are converted into soluble compounds, probably in the nature of sulphonic acid salts, and the cooking liquor remains substantially 55 neutral, and slightly alkaline to litmus, if and only if the monosulphite be used in sufficient quantities. Moreover, the cellulose of the fibers under such circumstances is either retained in or converted by the treatment 60 into, a form of cellulose not resulting from the treatment of the same raw materials by other reagents, or by monosulphite used in 65 inadequate quantities.

If the monosulphite be used in inadequate 70 quantities for the treatment of wood, as in the prior processes above referred to, an entirely different series of chemical reactions occurs, the cooking liquor becomes decidedly acid, and the advantages of my process are 75 lost. Again, if substantial quantities of additional reagents such, for example, as caustic soda on the one hand, or sulphurous acid on the other, be employed during the digestion (additional reagents being a feature of 80 most of the processes described in the prior patents and literature above referred to) the reaction partakes of the nature of the usual caustic or bisulphite processes, and the benefits of my invention are not attained. To 85 obtain my results the monosulphite cooking liquor must be used in sufficient quantities and under conditions adapted to produce substantially neutral soluble reaction products with the incrustations of the wood, through- 90 out the digestion.

The use of materially smaller percentages of monosulphite will result in acid reactions, and a much inferior, darker colored, weaker pulp.

For example, I have found that in the case of deciduous woods it is desirable to use upwards of 33 percent of sodium monosulphite to the air dry weight of the wood treated, and in the case of coniferous woods upwards 100

of 37% of sodium monosulphite. A substantial excess of monosulphite does not interfere with the process, but is of course wasteful. A slight excess of monosulphite over the minimum proportions is desirable as a safety factor. Other monosulphites may be used in corresponding molecular proportions. In the case of magnesium monosulphite so large an amount is not soluble in the amount of water it is desirable to employ; but I have found that if the requisite amount be added with the cooking liquor in undissolved form it will react during the digestion and produce the desired results. It is usually most convenient to use the sodium monosulphite.

Since the cooking liquor remains slightly alkaline throughout my process, it is possible to carry it out in unlined digesters, thus effecting a considerable saving. This cannot be done if smaller quantities of monosulphite be employed because of the acid reaction products formed in such cases.

According to my process the wood chips in the usual form are digested with the monosulphite cooking liquor containing, as above suggested, sufficient monosulphite to keep the process slightly alkaline throughout the digestion. The concentration of the liquor employed and the time and temperature used in the digestion may vary widely. The general rule is that stronger concentration and higher temperatures permit of shorter cooking times. In practice it has been found convenient to use a temperature of at least 170° C. and pressure of at least 100 lbs., and a concentration, for example, of 110 to 160 grammes of sodium monosulphite per liter of liquor.

The time of treatment is usually upwards of ten hours, but of course varies not only with the concentration and temperature employed, but also with the grade and condition of the wood, the type of digester used, etc.

The cooked fiber may be washed, separated, bleached, beaten, etc., in the usual manner. If, however, it is desired to bleach it, the following process can be conveniently employed with this particular fiber.

Chlorine gas is run into the wet pulp after thorough washing, or alternatively the pulp is treated with chlorine water. Agitation is advantageously used to promote the reaction. The chlorine is absorbed by the pulp forming addition products without the formation of hydrochloric acid, the bleaching liquor remaining neutral. In this respect the pulp from my process is peculiar, as other pulps will result in the formation of hydrochloric acid when treated with free chlorine. The chlorinated products can readily be washed out of my fiber by treatment with hot water. This is another advantage distinguishing my pulp from others. After wash-

ing, a slight treatment with bleaching powder solution, using for example about 2% on the weight of the pulp of 37 percent bleach, will turn the product snow white. The fiber resulting from the use of my process is light colored even before bleaching and snow white after bleaching. Not only is the yield of ultimate pure fiber by my process substantially greater than that obtained from the use of other reagents, but the fiber is much stronger and more flexible. It resists the destructive action of the beater more effectively than ordinary wood fiber, and like rag fiber tends when beaten to fray and produce "whiskers" which materially increase its matting qualities, and the strength and durability of paper made from it. In short, the fiber and paper resulting from my process resemble rag fiber and rag paper more than ordinary wood fiber and wood paper, and are quite superior in appearance, strength and durability to wood fiber and wood paper made by other processes.

It is obvious from the foregoing that many variations may be made in details of the process and product without departing from the spirit and scope of my invention.

What I claim is:

1. The process of digesting wood with a monosulphite cooking liquor, the monosulphite being used at a sufficiently high temperature and in sufficient quantities in proportion to the amount and character of wood treated to yield a spent liquor which is substantially neutral but alkaline to litmus at the end of the digestion and wood fibers characterized by unusual strength.

2. The process of digesting wood with sodium monosulphite cooking liquor, the sodium monosulphite being used at a sufficiently high temperature and in sufficient quantities in proportion to the amount and character of wood treated to yield a spent liquor which is substantially neutral but alkaline to litmus at the end of digestion and wood fibers characterized by unusual strength.

3. In the process of making paper the steps comprising digesting wood with a monosulphite cooking liquor, the monosulphite being used at a sufficiently high temperature and in sufficient quantities in proportion to the amount and character of the wood treated to yield a spent liquor which is substantially neutral but alkaline to litmus at the end of digestion and wood fibers characterized by unusual strength, washing the resulting fibers, and bleaching them by treatment with chlorine.

4. In the process of making paper, the steps comprising digesting wood with sodium monosulphite cooking liquor, the sodium monosulphite being used at a sufficiently high temperature and in sufficient quantities in proportion to the amount and character of the wood treated to yield a spent liquor which

is substantially neutral but alkaline to litmus at the end of digestion and wood fibers characterized by unusual strength, washing the resulting fibers, and bleaching them by treatment with chlorine.

5. In the process of making paper, the steps comprising digesting wood with sodium monosulphite cooking liquor, the sodium monosulphite being used at a sufficiently high temperature and in sufficient quantities in proportion to the amount and character of the wood treated to yield a spent liquor which is substantially neutral but alkaline to litmus at the end of digestion and wood fibers characterized by unusual strength, washing the resulting fibers and bleaching them by treatment with chlorine, and washing out the chlorinated products with hot water.

10 6. As a new product the herein described cellulose fiber produced by the digestion of wood with a monosulphite cooking liquor, the monosulphite present in sufficient quantity to yield by reaction with the woody incrustations a spent liquor which is substantially neutral but alkaline to litmus at the end of the digestion and such fibers being characterized by unusual strength.

7. As a new product the herein described cellulose fiber produced by the digestion of wood with sodium monosulphite cooking liquor, the sodium monosulphite present in sufficient quantity to yield by reaction with the woody incrustations a spent liquor which is substantially neutral but alkaline to litmus at the end of the digestion and such fibers being characterized by unusual strength.

8. As a new product the herein described cellulose fibers derived from wood but resembling in appearance, strength, flexibility and matting qualities, the cellulose fibers derived from rags, such fibers resulting from the cooking of wood with a monosulphite cooking liquor.

9. As a new product, the herein described strong, flexible, durable paper composed of wood fibers but resembling rag paper in quality, such wood fibers being produced by the digestion of wood with a sodium monosulphite cooking liquor.

10. As a new product the herein described pulp made from deciduous short fiber wood by digestion with a monosulphite cooking liquor, such fibers being of unusual strength and being capable of forming paper of unusual strength without admixture of long fiber pulp.

11. As a new product, paper made from the pulp of the preceding claim.

12. As a new product, paper produced from monosulphite pulp resulting from the cooking of wood with a monosulphite liquor, the fibers of such pulp having unusual strength and resistance to beating, and such

pulp having been subjected to beating to cause fraying of the fibers before the production of paper therefrom.

13. The method of producing paper which comprises cooking wood with a monosulphite cooking liquor to form fibers of unusual strength and resistance to beating, subjecting the resulting pulp to a beating operation to cause fraying of the pulp and to increase its matting qualities and the strength of the paper made therefrom, and forming paper of the resulting frayed pulp.

14. As a new product the paper resulting from the process of the preceding claim.

15. The method of producing paper from short fiber deciduous wood which comprises cooking the wood with a monosulphite cooking liquor to produce a short fiber pulp of unusual strength and resistance to beating, subjecting such pulp to a beating operation sufficient to effect fraying of the fibers, and forming paper from the resulting beaten and frayed fibers.

16. As a new product, paper produced in accordance with the process of the preceding claim.

VIGGO DREWSEN.

25

100

105

110

115

120

125

130

70

75

80

85

90